

# UNITED STATES PATENT OFFICE.

CHARLES M. REYNOLDS, OF SPARKS, NEVADA.

MANUFACTURE OF BRIQUETS AND OTHER ARTICLES.

1,103,078.

Specification of Letters Patent. Patented July 14, 1914.

Application filed April 28, 1914. Serial No. 834,979.

To all whom it may concern:

Be it known that I, CHARLES M. REYNOLDS, a citizen of the United States, residing at Sparks, in the county of Washoe and State of Nevada, have invented new and useful Improvements in the Manufacture of Briquets and other Articles, of which the following is a specification.

This invention relates to the manufacture 10 of compressed charcoal briquets from sawdust and other sawmill and timber waste, slabs or other refuse wood or organic vegetable substances, and the recovery of the volatile constituents of the organic matter, 15 such as alcohol, creosote, tar, turpentine or the like, freed therefrom by destructive distillation.

In carrying my invention into practice, the vegetable matter to be treated is first fed 20 into a stationary or rotary kiln or retort, in which it is wholly or partially carbonized. The volatile substances driven off from the material by this process of carbonization and destructive distillation are collected and 25 conveyed to suitable receptacles for condensation and the recovery of the by-products mentioned. Preferably the raw material, in a ground or comminuted state, is introduced into one end of the kiln or retort and dis- 30 charged from the opposite end thereof, the operation being practically continuous, and automatic in character. The carbon dis- charged from the kiln or retort, if not pre- 35 previously granulated or powdered is then gran- ulated or reduced to a suitably comminuted state, after which the material is fed into a mechanical mixer where it is combined while still hot with from three to five per cent. of crude oil, coal tar, pitch or any suit- 40 able one of the by-products as a binder, the ingredients being agitated and combined until thorough conglomeration ensues. The conglomérates are then fed from the mixer into any suitable type of briqueting machine, 45 in which they are formed under pressure into briquets of any desired size or shape. The briquets are then placed within a closed kiln or on a slowly traveling conveyer passing

through a highly heated kiln or chamber, to thoroughly dry or render the same porous, 50 hard and easy to handle, the heat driving off all of the remaining moisture and volatile matter contained in the mass through the addition of the binder. The moisture and volatile constituents may be carried off 55 and separated for the recovery of their component parts and the by-products resulting therefrom. If desired, the briquets when discharged from the second kiln or heating chamber may be cooled by an air blast or 60 other suitable cooling means, after which they are stored for use.

By this process of manufacture ordinary organic vegetable waste matter may be used with great economy in the production of 65 briquets, and superior briquets made, and at the same time all the volatile constituents of the material may be driven off and recovered, enabling greater economy of manufac- 70 ture to be obtained.

I claim:

1. The process of making briquets from wood waste, which comprises carbonizing said material, mixing the same with a suitable proportion of a volatile binder, comprising a part at least, of the material driven off during said carbonizing step, compressing the mixture into form, heating the same to a temperature sufficient to drive off the volatile constituents of the binder, and to 75 harden the briquets.

2. The process of making briquets from waste wood, which comprises carbonizing said wood, mixing therewith a suitable proportion of a volatile binder including the 85 tar driven off in said carbonizing step, compressing the mixture into form, heating the same to a temperature sufficient to drive off a part at least of the binder, and to harden the briquets.

In testimony whereof I affix my signature in presence of two witnesses.

CHARLES M. REYNOLDS.

Witnesses:

W. C. MARTIN,  
JAMES POLLOCK.